

## UNITED STATES PATENT OFFICE

2,590,013

## PLASTERBOARD, SCUFF RESISTANT PAPER LINER, AND PROCESS

Harry N. Huntzicker and John K. Wise, Evanston,  
Ill., assignors to United States Gypsum Company, Chicago, Ill., a corporation of Illinois

No Drawing. Application June 22, 1948,  
Serial No. 34,555

6 Claims. (Cl. 154—45.9)

## 1

This invention relates to scuff resistant paper and a process for producing same and more particularly to a building element, such as gypsum wallboard, having scuff resistant paper applied to one surface thereof.

Processes and apparatus for the manufacture of gypsum wallboard including a set-hardened gypsum core between a pair of paper liners are well known in the art. One such process comprises the steps of covering a high rosin size paper sheet with an aqueous slurry of gypsum to a predetermined depth, applying thereover a second paper sheet, and then permitting the slurry to set. The gypsum may contain a small quantity of starch which assists in the formation and maintenance of a strong bond between the paper sheets and the gypsum core in the final product. After the gypsum has set, the board is cut to size and kiln dried.

Gypsum wallboards prepared as indicated above are standard articles of commerce and are sold in large quantities. These boards are customarily erected by nailing them to conventional wood studs. However, in building construction, the joints between successive boards, that is, the places at which an edge of one board abuts against a corresponding edge of another board, have a tendency to be unsightly in the finished wall. Many different methods have been attempted in an effort to provide a cheap, feasible means of rendering the joints invisible in the final wall structure. The most widely used method has been to cover the joint with a filled aqueous adhesive cement, usually of the protein type, and embed therein a paper tape. After the adhesive cement has dried, an additional coat of the same or another adhesive is applied to smooth off the completed assembly. When this last mentioned adhesive has dried, the cemented area, which usually extends over each board face for several inches on either side of the joint, is sanded smooth. The result is a smooth, level, monolithic wall construction which is ready to be decorated.

The above mentioned system of wall construction has certain disadvantages when employing paper-lined plasterboards that are now available in commerce. When the final coat of the joint cement is sanded, it is practically impossible for the mechanic to avoid touching and sanding the adjacent paper surfaces of the wallboard with the sandpaper. Wherever such contact occurs, the surface of the paper of the wallboard is scuffed. This is very undesirable since subsequent painting tends to accentuate rather than to cover the scuff marks. A further undesirable feature is that the paper surface of the wallboard exhibits, when painted with oil paints, a marked tendency toward raising of the surface fibers. This also causes an unsightly appearance.

## 2

Factory sizing of finished plasterboards is impractical because the cost of handling the boards would be prohibitive. Furthermore, plasterboards emerge from the drying kilns at such a high rate of speed in lineal feet per minute that equipment necessary to size them at this point in the operation would be prohibitive in cost. The obvious expedient of applying a conventional size coat to the paper before the board is formed has proven to be a practical impossibility. This is so since at least a part of the water present in the initial aqueous plaster slurry must be removed from the core during the drying operation, thus necessitating that the vapors pass directly through the paper liners. For this reason the porosity of the paper must be very closely and carefully controlled prior to and during manufacture of the plasterboard. Experience has shown that application of conventional size coatings to the paper tends to seal the sheet and render it less porous. Thus when a gypsum wallboard is made from such a sheet, the water vapor in the core will have a tendency to blow the paper loose from the core during the drying cycle in the kilns.

It is therefore one object of this invention to provide an inexpensive, easy to apply sizing material capable of imparting to gypsum wallboard paper resistance to scuffing and fiber raising without substantially changing the porosity of the sheet.

A further object of this invention is the provision of a porous paper sheet having scuff resistant properties which is particularly useful in the manufacture of paper-lined gypsum boards.

A further object of this invention is the provision of a process of preparing paper having increased scuff resistance without imparting excessive brittleness properties to the paper.

A still further object of this invention is the provision of a paper-lined building element, such as plasterboard, which is resistant to scuffing when treated with sandpaper and which is capable of decoration, even on the sanded portions, with oil paints or water-thinned paints without bleeding or other adverse effect.

Further and additional objects will appear from the following description and the appended claims.

In accordance with this invention it has been discovered that scuff resistant properties may be imparted to paper by treating a paper sheet with a product prepared by heating together water, a polysaccharide from the group consisting of starches and dextrans, an aliphatic aldehyde and a nitrogen compound capable of reacting with the aldehyde to form a resin of the amine-aldehyde type. In accordance with one embodiment of this invention, an aqueous dispersion of starch or dextrin is heated, preferably above the gelat-

## 3

inization temperature, in the presence of urea and formaldehyde to form a reaction product which is thereafter used to treat a paper sheet, as will be hereinafter more fully described. The nature of the reaction between the starch or dextrin and the urea and formaldehyde is not clearly understood and it is not definitely known whether a well defined chemical reaction product actually forms during this heating treatment. However, it has been discovered that the heat treatment of these substances together in aqueous solution is necessary prior to the time that the solution is applied to the paper whereby to produce a paper having the desired scuff resistant properties and porosity. Simple mixtures of starch or dextrin and a previously formed urea-formaldehyde resin applied to a paper sheet exhibit insufficient penetration into the sheet, excessive embrittlement of the sheet, and markedly reduced porosity. Likewise treatment of a paper sheet with unreacted starch, urea and formaldehyde does not give the desired penetrability or the necessary degree of porosity that are obtained by the process and product disclosed and claimed herein.

In order more fully to explain the invention, reference will be made to the following examples which illustrate several particular embodiments thereof. However, it will be clear to one skilled in the art that this invention is not to be limited by the examples given but only by the scope of the claims appended hereto.

## Example 1

The following ingredients in the amounts indicated in parts by weight were thoroughly mixed:

|                |     |
|----------------|-----|
| Dextrin        | 120 |
| Urea           | 40  |
| Formalin (37%) | 216 |
| Water          | 290 |

The acidity of the resulting solution was adjusted to pH 5 to 5.5 and the batch was heated to 85° C. and held between 85° and 90° C. for 15 minutes. Thereafter the acidity was adjusted to about pH 7 and the heating continued for an additional 45 minutes. The resulting solution containing the reaction product or condensate of dextrin, urea and formaldehyde was applied in several concentrations (by diluting with water where necessary) to one surface of a chip paper of the type ordinarily employed in making gypsum wallboard. This paper was a highly rosin sized paper. The excess solution was then removed by a doctor blade and the sheet dried. The dried sheet was then baked to cure the condensate contained therein under conditions which simulate the high temperature drying of plasterboard in a commercial manufacturing process, 20 minutes at 250° F. being adequate. The resulting sheet was found to be remarkably resistant to scuffing and fiber raising when sanded with paper or emery cloth. Tests were made on the several papers with the results indicated in the following table:

| Per cent Solids in treating solution | Porosity of sheet before treatment | Porosity of sheet after treatment | Per cent Condensate in final sheet |
|--------------------------------------|------------------------------------|-----------------------------------|------------------------------------|
| 20                                   | 144                                | 126                               | 2.3                                |
| 15                                   | 154                                | 166                               | 1.8                                |
| 10                                   | 134                                | 136                               | 1.1                                |

The porosities reported in this example and in the succeeding examples were determined according to the standard Tappi method T-460m-44.

The porosity values refer to the number of seconds for 100 cc. of air to pass through a porous sheet under standard conditions. Accordingly the lower numbers in the table indicate a higher porosity.

## Example 2

The following ingredients in parts by weight were thoroughly mixed:

|                 |     |
|-----------------|-----|
| Oxidized starch | 40  |
| Urea            | 30  |
| Formalin (37%)  | 162 |
| Water           | 168 |

The mixture was heated at 85° to 90° C. for 90 minutes, the acidity of the solution being between pH 6 and 6.5. At the end of this time the acidity was adjusted to about pH 7 and the resulting condensate was applied to a gypsum board paper in several concentrations, dried and baked in the manner indicated above in connection with Example 1. Test results were tabulated as follows:

| Per cent Solids in treating solution | Porosity of sheet before treatment | Porosity of sheet after treatment | Per cent Condensate in final sheet |
|--------------------------------------|------------------------------------|-----------------------------------|------------------------------------|
| 25                                   | 170                                | 260                               | 2.8                                |
| 15                                   | 185                                | 190                               | 1.5                                |
| 10                                   | 160                                | 160                               | 1.2                                |

Although the porosity of the sheet treated with the 25% solution decreased from 170 to 260, this latter value is still well within the range required for gypsum board paper. The sheets were highly resistant to scuffing and fiber raising.

## Example 3

The following ingredients in parts by weight were thoroughly mixed:

|                |     |
|----------------|-----|
| Dextrin        | 90  |
| Urea           | 5   |
| Formalin (37%) | 27  |
| Water          | 278 |

This batch was heated at 85° to 90° C. for 15 minutes, the acidity ranging between pH 4.5 and 5. The acidity was then adjusted to about pH 7 and heating was continued for another 30 minutes. The resulting condensate was applied to gypsum board paper, dried and baked in the manner indicated in Example 1 with the following test results:

| Per cent Solids in treating solution | Porosity of sheet before treatment | Porosity of sheet after treatment | Per cent Condensate in final sheet |
|--------------------------------------|------------------------------------|-----------------------------------|------------------------------------|
| 20                                   | 120                                | 260                               | 3.0                                |
| 15                                   | 122                                | 180                               | 2.0                                |
| 10                                   | 130                                | 130                               | 1.3                                |

The sheets were found to be resistant to scuffing and fiber raising.

## Example 4

The following ingredients in parts by weight were thoroughly mixed:

|                      |     |
|----------------------|-----|
| Starch (90 fluidity) | 150 |
| Urea                 | 40  |
| Formalin (37%)       | 216 |
| Water                | 580 |

The acidity of the mixture was adjusted to pH 5 to 5.5 and it was heated at 85° to 90° C. for one hour. Thereafter the acidity was adjusted

## 5

to about pH 7 and the mixture was heated for an additional hour. This condensate when applied to gypsum board paper conferred, after being cured, good scuff resistance to the paper.

In order to explain the term "fluidity" as used in connection with the starch of this and the next example: "fluidity" is a term used by the starch industry to describe the extent of modification, degradation, or hydrolysis of the starch molecule. The test method for determining fluidity is carried out as follows: Five grams of starch are wet with 10 cc. of distilled water and 90 cc. of a 1% sodium hydroxide solution are added at 25° C. The solution is stirred for three minutes and allowed to stand for 27 minutes, after which the volume of solution which flows from a standard orifice in 70 seconds at 25° C. is measured. This volume is regarded as the "fluidity" of the starch (see Kerr, "Chemistry and Industry of Starch," 1944, at page 95).

## Example 5

In this example the following ingredients in parts by weight were employed:

|                                           |     |
|-------------------------------------------|-----|
| Acid hydrolyzed cornstarch of 90 fluidity | 150 |
| Urea                                      | 40  |
| Formalin (37%)                            | 216 |
| Water                                     | 580 |

A smooth paste was formed of the starch with some of the water and thereafter the remaining ingredients were added thereto in the amounts specified. The acidity was adjusted to pH 4.9 with dilute acetic acid and the batch was heated with stirring to 85° to 90° C. and held at that temperature for 60 minutes. Thereafter the acidity was adjusted to about pH 6.6 and the heating was continued for another 60 minutes whereafter the batch was allowed to cool. A portion of the resulting condensate was applied to a piece of high rosin size chipboard paper. After removal of the excess of the condensate by a doctor blade and baking, the surface of the sheet was found to be highly resistant to scuffing when rubbed with sandpaper or emery cloth. As a matter of fact, the abrasive actually smoothed rather than roughened the surface. The porosity and flexibility of the sheet were changed only slightly.

Another portion of the condensate formed as above indicated in this example was acidified to pH 4 with alum. This acidified solution was applied to another piece of chipboard paper in the manner indicated above with substantially the same results. A film cast from the acidified solution became hard and insoluble in water upon baking.

## Example 6

The following ingredients in parts by weight were thoroughly mixed:

|                |     |
|----------------|-----|
| Dextrin        | 150 |
| Urea           | 40  |
| Formalin (37%) | 216 |
| Water          | 580 |

The acidity was adjusted to pH 5.2 with acetic acid and sodium hydroxide. The batch was heated for one hour at 85° to 90° C. whereafter the acidity was adjusted to pH 7.44 with sodium hydroxide and the heating continued for an additional hour. Chipboard paper treated with the condensate in the manner previously indicated was found to be highly resistant to scuffing and fiber raising and the porosity of the paper was substantially unchanged. The condensate in this

## 6

example penetrated the paper a little more readily than the condensate of Example 5.

## Example 7

6 The following ingredients in parts by weight were mixed together:

|                 |     |
|-----------------|-----|
| Oxidized starch | 75  |
| Urea            | 10  |
| Formalin (37%)  | 27  |
| Water           | 685 |

The resulting mixture had an unadjusted acidity of pH 7.8. It was heated for one hour at 85° to 90° C. during which time the acidity drifted to pH 6.74. When applied to chipboard paper in the manner previously indicated, this condensate gave excellent scuff resistance with little change in sheet porosity.

## Example 8

20 The following ingredients in parts by weight were mixed together:

|                |     |
|----------------|-----|
| Dextrin        | 50  |
| Urea           | 30  |
| Formalin (37%) | 92  |
| Water          | 400 |

The mixture was heated for 90 minutes at 85° to 90° C., the acidity being about pH 6. The condensate was applied to paper in the manner previously indicated and when the excess was removed and the sheet baked, it showed excellent scuff resistance and practically no change in porosity.

## Example 9

35 The following ingredients in parts by weight were mixed together:

|                         |     |
|-------------------------|-----|
| Enzyme converted starch | 100 |
| Urea                    | 75  |
| Formalin (37%)          | 200 |
| Water                   | 700 |

The acidity of the resulting batch was adjusted to about pH 7 and the batch was then heated for two hours at 85° to 90° C. Paper treated with this condensate and baked was resistant to scuffing and substantially unchanged in porosity.

It will be apparent from the foregoing examples that the amount of condensate applied to the surface of the paper may vary within wide limits. It is preferred, however, that the conditions be controlled so that the final paper sheet product contains between about 0.5 and about 5.0 per cent by weight of condensate, preferably between about 1.0 and 3.0 per cent. It is preferred for proper porosity control that the condensate penetrate into the surface of the sheet at least to some extent. Penetration may be expedited by rolling or calendering the sheet. Obviously the bulk of the condensate is close to the surface and in the case of manila papers the manila liner may contain 35 per cent or so of condensate with practically none in the filler plies even though the condensate may be present in amounts of 5 per cent or less of the total weight of the sheet.

In commercial practice it is preferred to apply the condensate to the highly rosin sized paper sheet directly on the paper machine before it enters the calender stacks. In this manner uniform penetration is made easier and the condensate appears to enhance the finish of the sheet on calendering. However, it will be apparent that the other methods of application will occur to those skilled in the art.

The paper that has been treated in the manner indicated in the previous paragraph is ready for application as a liner to gypsum board. This may be effected in any desired manner such as those commonly in practice now in the industry and as indicated in the foregoing. After the paper-lined gypsum sheet has set, the gypsum board is then dried out in suitable kilns maintained at high temperature. The heat treatment in the kilns serves in a measure to bake or 5 cure the condensate directly within the paper sheet, thereby rendering the sheet scuff resistant. This corresponds to the baking step indicated in the previous examples. It is at this point in the manufacture of the gypsum board that it is most desirable for the porosity of the paper sheet to be maintained since in the drying kilns or ovens water vapor must escape through the paper liners. If the liners are 10 insufficiently porous, then they will have a tendency to be blown loose from the gypsum core during the drying cycle. In the commercial kilns now in use, the air intake temperature may range between 250° and 500° F. and accordingly the paper liners must permit of the ready escape 15 of steam or water vapor therethrough during the drying period.

As previously indicated, it is an important feature of this invention that the polysaccharide (i. e. starch or dextrin) be heat-treated in the presence of water and the urea and formaldehyde prior to application to the paper sheet. In connection with this cooking procedure, there do not appear to be any critical factors other than those which will permit the proper reaction between the several ingredients to take place. As is well known in the resin art, the speed and extent of reaction will depend upon the inter-relationship of time, temperature, acidity and concentration factors. However, it is preferred to heat or cook the several ingredients at a temperature which is above the gelatinization temperatures of the starch or dextrin employed. The range of 85° to 90° C., as indicated in all of the examples, is suitable. As previously indicated, if the several ingredients are not pre-cooked or otherwise prereacted prior to the time that they are applied to the paper, it is substantially impossible to obtain proper penetration. The preheating or prereacting of the several ingredients breaks down the gel characteristics of the starch or dextrin, and a viscous flow is permitted which will permit at least a portion of the composition to penetrate into the surface of the paper.

It will be apparent from the foregoing that any type of starch or dextrin may be employed in accordance with this invention. It is preferred to use a converted starch to improve penetration so that the proper amount of condensate will be carried into the sheet. As previously indicated, the amounts of condensate present in the final sheet may be as high as 5 per cent of the total weight of the sheet, the preferred range being between about 1 and 3 per cent. It will also be apparent that the urea may be replaced in whole or in part with other nitrogen-containing organic compounds known to react in an analogous fashion with aldehydes. Such materials may include thiourea, melamine, dicyandiamide, biuret, formamide, acetamide, ethanolamine, diethylamine, sulfamates and the like. As a matter of fact, while urea is preferred, any amine or amide may be employed which is capable of reacting with an aldehyde to form a resin

commonly referred to as one of the amine-aldehyde type. Likewise this invention is not limited to the use of formalin as specified in the foregoing examples. Other sources of formaldehyde, such as paraformaldehyde, trioxymethylene, hexamethylenetetramine, etc. may be employed. Also other aldehydes which may react with the amine and/or amide, such as acetaldehyde, butyraldehyde, glyoxal, furfural, etc. may be employed as complete or partial replacements for formaldehyde.

As will be apparent from the foregoing examples, the treated paper may be prebaked to set the resin and thereafter the paper may be applied to a gypsum board as a top cover sheet.

While several particular embodiments of this invention are shown above, it will be understood, of course, that the invention is not to be limited thereto, since many modifications may be made, and it is contemplated, therefore, by the appended claims, to cover any such modifications as fall within the true spirit and scope of this invention.

We claim:

1. A decorative plasterboard having secured to at least one surface thereof a porous, highly sized calendered paper sheet having scuff-resistant properties, said sheet containing in gradually diminishing quantities from the exposed surface thereof in an amount between about 0.5 and about 5 per cent by weight of the sheet, a heat-cured pre-formed heat reaction product of water, a polysaccharide selected from the group consisting of starches and dextrans, a compound selected from the group consisting of aliphatic amines and amides, and an aldehyde, the molar ratio of said aldehyde to said compound being within the range of about two to one and about four to one.
2. The plasterboard recited in claim 1 wherein said compound is urea and wherein said aldehyde is formaldehyde.
3. A porous, highly sized calendered paper sheet suitable for use as a gypsum wallboard paper liner and having scuff-resistant properties which contains in gradually diminishing quantities from one surface thereof in an amount between about 0.5 and about 5 per cent by weight of the sheet, a heat-cured pre-formed heat reaction product of water, a polysaccharide selected from the group consisting of starches and dextrans, a compound selected from the group consisting of aliphatic amines and amides, and an aldehyde, the molar ratio of said aldehyde to said compound being within the range of about two to one and about four to one.
4. The porous paper sheet recited in claim 3 wherein said compound is urea and wherein said aldehyde is formaldehyde.
5. A process of treating a highly sized porous paper suitable for use in the manufacture of paper-lined gypsum wallboard to impart scuff-resistant properties to said paper without essentially changing the porosity thereof which comprises applying to one surface of said sized paper an aqueous solution of a heat reaction product of water, a polysaccharide selected from the group consisting of starches and dextrans, a compound selected from the group consisting of aliphatic amines and amides, and an aldehyde, the molar ratio of said aldehyde to said compound being within the range of about two to one and about four to one, the amount of said solution applied to said paper being sufficient to deposit on said surface solid reaction product

in an amount equal to between about 0.5 and about 5 per cent by weight of said paper, and thereafter calendering said paper whereby said reaction product is distributed in the paper in a gradually decreasing concentration from the surface thereof.

6. The process recited in claim 5 wherein said compound is urea and wherein said aldehyde is formaldehyde.

HARRY N. HUNTZICKER.  
JOHN K. WISE.

## REFERENCES CITED

The following references are of record in the file of this patent:

## UNITED STATES PATENTS

|           |              |               |
|-----------|--------------|---------------|
| Number    | Name         | Date          |
| 2,212,314 | Bauer et al. | Aug. 20, 1940 |

|   | Number    | Name          | Date          |
|---|-----------|---------------|---------------|
| 5 | 2,246,635 | Moller        | June 24, 1941 |
|   | 2,338,602 | Schur         | Jan. 4, 1944  |
|   | 2,352,553 | Lefebure      | June 27, 1944 |
|   | 2,452,054 | Jones         | Oct. 26, 1948 |
|   | 2,496,440 | Caesar et al. | Feb. 7, 1950  |

## FOREIGN PATENTS

|    | Number  | Country       | Date          |
|----|---------|---------------|---------------|
| 10 | 539,331 | Great Britain | Sept. 5, 1941 |
|    | 57,967  | Netherlands   | Aug. 15, 1946 |

## OTHER REFERENCES

15 "The Use of Urea-Formaldehyde Resin for Waterproofing Starch Used in Corrugated and Solid Fiberboard Production," by Philip B. Taft, published in the Paper Trade Journal, Oct. 15, 1942, pages 30-32 or Tappi Sections 206-208.